

## UNITED STATES PATENT OFFICE

DONALD K. PATTILLO, OF DOVER-FOXCROFT, MAINE; GEORGE E. CORSON, OF CLINTON, IOWA; AND HERBERT L. THOMPSON, OF NORWOOD, MASSACHUSETTS, ASSIGNORS TO CLINTON CORN SYRUP REFINING COMPANY, OF CLINTON, IOWA, A CORPORATION OF IOWA

## PAPER-MAKING PROCESS

No Drawing.

Application filed April 25, 1931. Serial No. 532,990.

This invention relates to paper-making processes and especially to those processes which involve the addition to the paper stock of amyloseous bonding material. The term 5 amyloseous bonding material referred to in this invention pertains to various starches, starch conversion products, dextrines, gums and oxidized starches or derivatives thereof which upon addition to a cellulose fibre effect 10 an increased bonding by reinforcing or strengthening of the already hydrated or gelatinized fibres.

It is one of the objects of this invention to provide an improvement in paper-making processes by which a greatly increased retention of the amyloseous bonding material is secured over what is possible in the paper-making processes as now practiced.

This increased retention of the amyloseous bonding material results in a better paper product, and as applied to paper it results in a paper which has an increased bursting and tensile strength, a greater folding endurance, 20 greater tearing resistance, improved sheet formation, improved surface finish, decreased porosity, increased density, increased opacity, increased dielectric strength, decreased elongation, decreased formation of pin-holes, increased fibre hydration or gelatinization and increased twisting strength, increased wet strength, decreased absorptive capacity and increased flexibility besides other improved characteristics.

The terms "paper" or "paper product" as referred to in this invention pertains to those cellulosic products formed in a continuous web by any of the generally accepted methods of manufacture, as for example, writing, bond, ledger, cover, book, tissue, wrapping, 35 coating, paper boards, in its many modifications and forms, insulating paper, twisting, roofing and saturating felts, composition and wall boards, and, in fact, any paper or paper board or specialty product in the many forms 40 in which these types of products are produced.

According to the present practice it is customary to add the amyloseous bonding material to the beater. Experiments have 50 shown that when the amyloseous bonding

material is added to the paper stock in the beater there will result a relatively low retention of the bonding material in the finished product. In fact, this retention varies from 10% to 40%, the remainder of the bonding 55 material being lost to the process.

In a paper-making process the beater operates to separate the fibre bundles and to secure hydration by mechanical means. If the amyloseous bonding material is introduced into the beater the action of the beater promotes particle break down of the bonding material due to the passage of the material between the beater roll and the bed plate thus decreasing markedly its bonding 60 effect and the retention of the particles of bonding material on the cellulose fibres, contrary to the general accepted theory. So, too, this repeated contact of the beater roll fly-bars and bed plate bars on the cellulose 65 fibres prevents the adhesion of the particles of bonding material except in limited amounts.

Our work has shown that in a closed system where the particles of amyloseous bonding material are recirculated constantly to come in repeated contact with the cellulose 75 fibres that the amount of retention secured is practically constant under a given set of conditions.

According to the present invention the amyloseous bonding material is added to the paper stock subsequent to the beating operation but prior to the formation of the paper web. Our experiments have shown that where the amyloseous bonding material is introduced in this manner there will be a very greatly increased retention of the material added, the retention in some cases being 85 nearly 100%. Such increased retention improves the quality of the finished product in the particulars mentioned above.

By introducing the amyloseous bonding material subsequent to the beating operation 95 the break down of the particles of the bonding material is avoided and consequently practically all of said particles readily adhere to and remain attached to the hydrated or gelatinized fibres of the fibre-water mix- 100

ture and thus become effective in bonding the fibres together.

Fibre-water mixture or fibre-water flow as referred to in this invention pertains to the process flow of cellulose fibre from the beater chest to the paper machine wire. Generally the amount of cellulose in the fibre water or fibre-water flow varies from 75 pounds to 500 pounds per 1000 gallons of water. In distinction to this the return or white water flow has a much lower fibre content, seldom exceeding 5 pounds of fibre per 1000 gallons of water. In further distinction a raw water line is that which supplies water used as make up or supply water and contains no fibre.

Our work has shown that the addition of amylose bonding material particles by this new process effects great improvement in the retention secured and that the same retentions are secured regardless of whether the process is in operation on an open, a closed or a partially closed system. The increased adherence of the amylose bonding material particles to the gelatinized fibres induces an apparent hydration or gelatinization resulting in the effects above mentioned.

It is thus seen that this process of addition is in effect a physical-chemical combination of the amylose bonding particle with the hydrated or gelatinized fibre as differentiated from a mechanical combination of the disrupted amylose bonding material particle and the unhydrated fibre in the beater process. This increased hydration or gelatinization may be due in part or in whole to the added gelatinizing effect of the amylose bonding material particle or may be due in part or in whole to the effect of this particle addition on the hydrated or gelatinized fibre but we do not distinguish between an actual cellulose hydration and a combination of chemical and physical cellulose hydrations and so refer to this increased hydration as an apparent added hydration of the cellulose fibre.

It is thus obvious that with an increased apparent hydration of the cellulose fibre modifications can be made in the mechanical preparation of the fibre to compensate for the added effects induced by the addition of the amylose bonding material particles. We have found that by this process it is possible to reduce the power loadings on the Jordans and engines or to reduce the time of fibre preparation in the beating engines to effect noteworthy power savings in the preparation of the fibre for paper-making purposes, and yet to produce a paper equal or better in all characteristics to paper made by any prior processes.

Our work has further shown that instead of reducing power loading on the Jordans or time of preparation in the beaters it is possible to substitute an inferior and less ex-

pensive fibre for the more expensive fibres used in the furnish for the reason that this added apparent hydration makes possible the production of sheets with equal or better characteristics from inferior cellulose fibre than can be produced under present practice with more expensive raw materials.

Our work has further shown that the actual amount of amylose bonding material retained in the finished product determines many of the physical characteristics of the paper product as discussed above. It is apparent, therefore, that the control of the amount of amylose bonding material in the finished product will control to a more or less degree the improved physical characteristics of the paper produced and with a constant retention of amylose bonding material as in this process of addition the characteristics of the paper product can be more definitely predetermined and controlled by varying the amount of amylose bonding material added in the methods above described.

This process is particularly adaptable to the manufacture of specialty papers wherein one or more characteristics of the finished product enhances the value of the paper for conversion use. It is possible by this process to more or less control any or several of these paper characteristics to produce a superior sheet of paper for a particular purpose.

Our work has shown that if increases in the physical strength characteristics of the paper are desired we can obtain such strength increases in definite relation to the amount of amylose bonding material added and that by so doing we can evolve paper products that are not possible under present day practices. For example, the addition of amylose bonding material particles by this new process produces a sheet of bag paper having an increased bursting strength of approximately 30%, a decreased elongation of approximately 30%, and a closer formation with the same or lower porosity, which characteristics contribute largely to the quality of bag paper. Under present operating practices it is not considered practical or possible to effect these changes in bag paper which are brought about by the effect of amylose bonding material particles in controlled amounts by the process above described. Other possibilities are apparent and the above is cited as a definite example of what can be accomplished in the manufacture of paper or paper specialties.

In the manufacture of paper products on multi-cylinder machines the adhesion of the various plies or cylinder sheets is of great importance. In the ordinary process of paper making this ply adhesion is controlled more or less by a control of the hydration

of the cellulose fibres making up the different cylinder sheets. It is obvious, therefore, that such adhesion will vary with different fibres used and our work has shown that in 5 many cases ply adhesion so controlled is very unsatisfactory. This process greatly increases ply adhesion on multi-cylinder machines for reasons that with the greatly increased retention of the amylose bonding 10 material particles the top and bottom surfaces of each cylinder sheet have in effect a layer of gelatinized bonding particles which adhere to adjacent layers of the paper web from adjoining cylinders to effect a greatly 15 increased bonding strength between the different cylinder sheets, which bonding strength is further increased by the action of the higher temperatures in the paper drying operation and by the subsequent compression of the paper in passing through the calendar stacks.

In some types of paper or paper board manufacture the product is made on a wet machine and the finished sheet is picked up 20 from a make-up roll in sheet form. As the sheet of board from the wet machine is not heavy enough in itself a great many sheets are imposed on each other to form the finished product and the adhesion between the 25 sheets is of great importance in the strength and quality of the finished board. With this process such sheet adhesion is greatly increased as we have discussed in regard to multi-cylinder machine operation.

30 It is a general practice today in paper mills to chlorinate the paper mill system in whole or in part for the purpose of slime prevention and sterilization of the flow and product. Our work has shown that such a chlorination process removes from the paper mill system certain organic buffer salts and other organic solubles which if present retard or decrease slightly the effects produced by this 35 process of amylose bonding material addition. Our work has shown, therefore, that while this process is particularly effective in both chlorinated and unchlorinated systems the effects produced in a chlorinated system 40 are slightly greater than those secured in an unchlorinated system. It is sometimes customary in the chlorinating process to use a combination of ammonia and chlorine and designate this sterilizing action as a "chloramine" process. It is apparent that the same 45 benefits will be found in the operation of this process in a "chloramine" treated system as in a chlorinated system.

50 As stated above the amylose bonding material which is contemplated by this invention may be various starches, starch conversion products, dextrines, gums and oxidized starches or derivatives thereof. The amount of any particular amylose bonding material or combination of these materials used

will depend upon the characteristics desired in the finished product.

It will be found from the above that this invention is equally applicable to so-called "open systems" or to so-called "closed or partially-closed systems." In the open system all the white water is lost to the process while in the closed or partially-closed system some or all of the white water is returned to the fibre-water mixture either at the beater or at any point between the beater and the paper machine wire.

70 In an open system process the amylose bonding material may be introduced into the fibre-water flow at any desired point between the beater and the paper machine wire, that is, it may be introduced into the paper stock at the Jordan headbox, or, and preferably, 75 at a point subsequent to the Jordan headbox.

80 As applied to a closed or partially-closed system the amylose bonding material may be introduced into the white water return flow at any point subsequent to the white water collecting box or between the paper machine wire and collecting box but prior to 85 the addition of the white water to the fibre-water flow. The addition of the amylose bonding material may also be made through any raw water line on either an open or closed or partially-closed system prior to its addition to the fibre-water flow.

90 Our work has shown that the amylose bonding material is best added continuously either in a dry state by means of a dry chemical feeder or in a solution or suspension form 100 by means of suitable equipment for introducing the material in the solution or suspension form. It is possible also to add the amylose bonding material semi-continuously and to compensate for the lack of continuity in 105 feed by the proper control of the rate of feed after a lapse in feeding or by the subsequent mixing of treated and untreated cellulose fibre in a suitable chest or tank with proper agitation to produce the same effects as if 110 the amylose bonding material had been added in continuous flow.

115 We claim.

1. That improvement in the process of making paper to improve its physical characteristics which consists in mechanically hydrating the fibres by a beater operation, flowing the mixture to a paper making machine and adding an amylose bonding material to the mixture at a point between the beater 120 and the paper making machine thereby securing an increased retention of the bonding material in the finished paper over that obtained by adding the bonding material to the beater.

125 2. That improvement in the process of making paper which consists in subjecting the fibre-water mixture to the operation of a beater to hydrate the fibre, flowing the beater-treated fibre-water mixture to a paper mak- 130

ing machine on which the paper is made and adding to the fibre water flow continuously and in regulated quantities an amylose bonding material thereby securing a greater 5 retention of the bonding material and consequent improved physical characteristics in the finished paper over that obtained by adding the bonding material to the beater.

3. That improvement in the process of making 10 paper which includes a white-water return flow delivering to the fibre-water flow at a point subsequent to the beating operation, which improvement consists in adding to the white-water return flow an amylose bonding 15 material thereby securing an increased retention of the bonding material and consequent improved physical characteristics in the finished paper over that where the bonding material is added in the beater.

20 4. That improvement in the process of making paper which consists in adding amylose bonding material to the fibre-water flow between the beater and the paper making machine through the raw water supply line, 25 thereby securing an increased retention of bonding material and consequent improved physical characteristics in the finished paper.

In testimony whereof, we have signed our names to this specification.

**30** DONALD K. PATTILLO.  
GEORGE E. CORSON.  
HERBERT L. THOMPSON.

**35**

**40**

**45**

**50**

**55**

**60**

**65**